

No. 856,630.

PATENTED JUNE 11, 1907.

J. S. GREEN.

TURBINE BLADE AND VANE.

APPLICATION FILED JAN. 2, 1907.



WITNESSES:

*B. B. Davis*

*E. H. McCallister*

INVENTOR.

*J. S. Green*

# UNITED STATES PATENT OFFICE.

JONATHAN S. GREEN, OF PITTSBURG, PENNSYLVANIA, ASSIGNOR TO  
THE WESTINGHOUSE MACHINE COMPANY, A CORPORATION OF  
PENNSYLVANIA.

## TURBINE BLADE AND VANE.

No. 856,630.

Specification of Letters Patent.

Patented June 11, 1907.

Application filed January 2, 1907. Serial No. 350,417.

*To all whom it may concern:*

Be it known that I, JONATHAN S. GREEN, a citizen of the United States, and a resident of Pittsburg, in the county of Allegheny and State of Pennsylvania, have made a new and useful invention in Turbine Blades and Vanes, of which the following is a specification.

This invention relates to blades and vanes for elastic fluid turbines.

In the manufacture of elastic fluid turbines, various metals have been used for the blades and vanes thereof, such as copper, bronze, nickel, nickel alloys, iron and steel. It has also been proposed to galvanize, sherardize, plate or enamel blades for the purpose of obtaining a satisfactory core portion and a satisfactory cover or envelop.

Blades produced from any of the single or alloyed metals heretofore used, or protected blades produced by any of the methods heretofore used, so far as I am aware, have proven unsatisfactory in use for various reasons. The rotors and stators of elastic fluid turbines, especially those of any size, are made of steel or iron, and with the temperature changes encountered as well as the centrifugal forces, in producing a satisfactory turbine blade or vane we are confronted with other problems aside from the deterioration of the blade or vane from erosion and corrosion. It has been found that steel blades, while satisfactory in many respects, cannot be used on account of their deterioration from both erosion and corrosion: copper, bronze and blades formed from other alloys, while they do not deteriorate as steel blades do, are unsatisfactory owing to the difference in the co-efficients of expansion between them and the blade or vane holding element of the turbine, such as the rotor and stator. Plated, galvanized and enameled blades such as heretofore proposed are unsatisfactory because of the difference of the co-efficients of expansion between the protective cover and the blade proper, and further, because of the liability of the cover to chip or crack off from other causes encountered in the operation of turbines.

An object of this invention has, therefore, been to produce a turbine blade or vane, the core or major portion of which will have the same co-efficient of expansion as the blade or

vane holding element, and which is provided with a protective covering of such metal as will withstand the erosive and corrosive action encountered, and produced in such a manner that the cover or armor cannot crack or chip off.

A further object has been to produce a turbine blade or vane, the core or major portion of which is formed from metal having the same coefficient of expansion as the blade or vane holding element, with a protective armor or sheath welded to the core or major portion.

In the drawings accompanying this application and forming a part thereof: Figure 1 is a perspective view of a fragmentary portion of a blade or vane holding element of a turbine showing a portion of a row of blades or vanes mounted therein; Fig. 2 is an end view of two of the blades or vanes of a turbine showing suitable means for lashing their outer or free ends together.

Each blade or vane preferably comprises a drawn steel core 3, which is provided with a sheath or cover 4 welded thereto and preferably formed of copper. The rotor element of the turbine is provided with slots 5 in which the blades are mounted. Any suitable method of mounting the blades may be employed, but in the method illustrated in the drawings the blades are inserted in the slot 5 and secured in place by means of calking pieces 7, which are inserted in the slot between the blades and are transversely expanded by pressure, so as to grip the walls of the slot and the faces of the end portions of the adjacent blades. The calking pieces 7 are made of the same material as the rotor element and the cores of the blades so that the several elements of the organized structure will contract and expand, due to temperature variations, in the same degree. Such a condition is essential, in order that the blades will remain tight in the slot. The vanes are mounted in the same manner in slots 5 which are formed in the stator. The outer or free ends of the blades or vanes, in each row, are connected together in sets by means of a suitable binding wire 8, which is inserted through holes punched near the outer ends of the blades or vanes.

I have shown the same form of binding wire as disclosed in United States Letters

Patent No. 791,837, issued to Charles E. Sweet on June 6, 1905, but instead of making the wire, as shown in said patent, of one metal; I preferably make mine of two metals, 5 that is, I provide a steel or iron core for the body portion of the wire and a protective covering, preferably of copper, for the fin portion, which covering extends to form the fin 11, which is sheared off between adjacent 10 blades or vanes to form spacers as described in said patent.

In manufacturing the blades or vanes which comprise my invention, an ingot or billet of mild steel or iron is provided with a 15 protective metal cover or envelop, which is welded onto it by a process which has proven to be effective. The billet with its protective covering is worked as an integral mass and is eventually drawn or rolled into strips of the 20 desired blade section and cut into proper blade lengths. When the blades are formed in this manner the ends of the cores are unprotected, but it has been found by experiment that the erosive and corrosive action 25 of the steam and water does not affect the core at the end of the blade when the ends only are exposed.

During the operation of drawing the blades the protective metal utilized is worked and 30 compressed between the hard steel die and the hard blade core until it becomes homogeneous. When single or alloy metal blades or vanes having a different co-efficient of expansion from the blade or vane holding elements are used, several difficulties arise. 35 If the co-efficient of expansion of the metal from which the blade is made is less than that of the holding element, under the high temperatures encountered in operating the turbine, the blades will loosen and become dislodged by the centrifugal force encountered. 40 If the co-efficient of expansion of the blade metal is greater than that of the holding element, under the temperatures encountered in 45 operation, those portions of the blades lying below the surface of the mounting element become crushed or compressed beyond the elastic limit of the metal, and with a decrease in temperature the blades become loose. With 50 blades manufactured in accordance with this invention, however, having a steel or iron core of the same co-efficient of expansion as the mounting element, if the mounting element is made of steel or iron, the protective 55 cover, owing to its thinness, does not cause any harmful result, for the core or major portion of the blade will expand and contract under varying temperatures as though no cover were present. The welding process holds the 60 cover securely in place on the core and there

is no tendency to chip, crack or peel off when subjected to the varying strains occasioned by the temperatures encountered. The binding wire 8 is formed in substantially the same manner, the dies for forming it being of 65 different cross section and provided with the necessary slot for forming the projecting fin.

Various and other methods may be employed in the manufacture; for example, after the billets are worked down to the proper 70 size the blades may be formed by drop forging or stamping and various thicknesses of protective metal may be employed. Each blade may be provided with a protective covering which is separately welded thereto, although this would be a tedious and expensive 75 operation.

Having thus described my invention, what I claim as new and useful and desire to secure by Letters Patent is:

1. In combination with a turbine blade holding element, a turbine blade, the core or major portion of which is formed of metal having substantially the same coefficient of 80 expansion as the metal of said element and a relatively thin sheath or cover welded to said core and formed of metal adapted to withstand the erosive and corrosive effect of the working fluid.

2. In combination with a turbine blade holding element, a turbine blade, the core or major portion of which is formed of a metal having substantially the same coefficient of expansion as the metal of said element and a relatively thin sheath or cover of protective 95 metal welded thereto.

3. In combination with a turbine blade holding element, a turbine blade, the core or major portion of which is formed of a metal having substantially the same coefficient of 100 expansion as the metal of said element and a relatively thin sheath of copper welded thereto.

4. In combination with a steel or iron blade holding element, a turbine blade comprising a core portion formed of steel or iron and a relatively thin sheath or cover of copper welded thereto.

5. In combination with a steel or iron blade holding element, a turbine blade comprising a core portion formed of steel or iron and a relatively thin sheath of protective metal welded thereto.

In testimony whereof, I have hereunto subscribed my name this 29th day of December, 1906.

JNO. S. GREEN.

Witnesses:

CHARLES W. MCGHEE,  
E. W. McCALLISTER.